

## UNITED STATES PATENT OFFICE.

LESTER KIRSCHBRAUN, OF EVANSTON, ILLINOIS.

## COATED WATERPROOF SHEETING.

No Drawing. Application filed February 1, 1919, Serial No. 274,495. Renewed January 27, 1923.

*To all whom it may concern:*

Be it known that I, LESTER KIRSCHBRAUN, a citizen of the United States, residing in the city of Evanston, county of Cook, and 5 State of Illinois, have invented certain new and useful Improvements in Coated Waterproof Sheetings, of which the following is a specification.

This invention relates to improvements in 10 coated waterproof coverings and process of making same, such, for example, as roofing, and has among its salient objects, to provide a waterproof felted sheet, to which is applied a fibre containing adhesive coating; 15 to provide a product in which the body or felted portion is preferably waterproofed simultaneously with the formation of the sheet, although in certain cases the body portion may consist of ordinary saturated 20 felt to which is applied the fibre containing coating; to provide a product which permits of the use of relatively low melting point asphalt as a coating; to provide a product in which the coating has a maximum 25 stability and in which the asphalt or bitumen is re-inforced against flowing by the fibrous constituents; to provide a product in which very cheap fibre of many different kinds can be used, and, in general, 30 to provide an improved product and process of the character referred to.

Describing now the preferable way of forming the product of the present invention, I make an aqueous mixture of water 35 and an emulsifying agent, such, for example, as a clay containing a sufficient percentage of colloidal particles. To this mixture, and while it is in a heated condition, is added an adhesive binder while in liquid form, 40 such as melted asphalt or analogous bitumens or pitches. The binder is thoroughly amalgamated with the emulsifying agent and water so as to form an emulsified matrix in which the binder is in the internal 45 phase and the emulsifying agent and water in the external phase. This matrix is then intimately mixed with the fibre in a water vehicle. The matrix above referred to may consist, by weight, of fifty parts binder, forty parts water and ten parts clay. 50 This mixture, with the fibre added, may be then passed over an ordinary paper or felt machine. As the sheet is formed, the water dries out and the emulsion is broken, and 55 the bitumen becomes adhesive and intimate-

ly unites with the fibre. The proportion of ingredients in the finished sheet may be as follows: fifty-five per cent of asphalt, eleven per cent of clay and thirty-four per cent of fibre. 60

After this sheet is formed, as stated, the coating is applied, preferably after the sheet passes over the last drying rolls of the paper machine. The coating mixture, 65 after being formed in the manner herein-after described, may be applied in the same way as asphalt coating is applied to ordinary saturated felt. The coating in the present invention, as heretofore stated, consists of bitumen and fibre. Preferably, the 70 coating consists of a mixture of an emulsified matrix and fibre formed in the manner heretofore described, except that a much less percentage of fibre is used. For example, the mixture may consist of 10 per cent of fibre, the remainder being asphalt and clay. The emulsion is formed for the 75 reason that the coating can thus be applied cold, but it is not desired to felt the coating; rather, the fibre may be said to more or less float through the asphalt, producing thereby a fibred asphalt coating. For example, a coating of this character may, in some cases, use asphalt for as low as 140 80 melting point, whereas, ordinarily, from 200 85 to 260 melting point asphalt is used; by melting point of the asphalt is meant that temperature at which the asphalt begins to melt when subjected to heat. Various fibres 90 may be used in this coating, such as cheap fibres ordinarily not suitable for making good paper. After the coating is applied, the sheet is run over drying rolls to remove the water. The bitumen then acts in the manner heretofore described. As the water 95 is driven out, the heated bitumen becomes plastic and a granular facing can then be applied to the adhesive coating.

I claim as my invention:

1. A process of making a waterproof covering consisting in forming a waterproof fibrous sheet, and then applying bitumen coating thereto in an aqueous vehicle containing an emulsifying agent and a minor percentage of fibre. 100

2. A process of making a waterproof covering consisting in forming a waterproof fibrous sheet, and then applying bitumen coating thereto in an aqueous vehicle containing an emulsifying agent and a minor 105 110

percentage of fibre, and finally apply a granular facing to the coating while the latter is in heated condition.

3. A process of making a waterproof covering, consisting in forming a mixture of emulsified bituminous matrix and fibre into a sheet, drying the sheet and permitting the

bituminous ingredient thereof to unite with the fibre, and then applying a mixture of bituminous emulsified matrix and a fibre <sup>10</sup> to the sheet in an aqueous vehicle and drying out the water.

LESTER KIRSCHBRAUN.